

## United States Patent Office

3,111,358

Patented Nov. 19, 1963

1

3,111,358

## HYDRAZINE SALT FOR ACTIVATION AND STABILIZATION OF CHLORITE BLEACH FOR CELLULOSIC TEXTILES

Richard L. Doerr, Orange, Conn., assignor to Olin Mathieson Chemical Corporation, a corporation of Virginia  
No Drawing. Filed Apr. 14, 1961, Ser. No. 102,966  
16 Claims. (Cl. 8—108)

The present invention relates to improvements in bleaching cellulosic textiles and textile fibers using aqueous solutions of chlorites.

The present invention is useful in bleaching cotton goods of all kinds, including cotton, linen, jute, hemp and other textile fibers consisting essentially of cellulose as well as cellulose regenerated from a viscose solution. Also included and successfully bleached by the process of the present invention are blended textiles, such as blends of cottons and nylon, cottons and synthetic polyester fibers, cotton and polyacrylonitrile and other blends containing even minor proportions of cellulosic fiber. All such textiles are intended to be included in the term "cellulosic textiles and textile fibers" as used in the present specification and claims.

The bleaching agents normally used in the United States are alkaline hydrogen peroxide, hypochlorite, and chlorites. Chlorite bleaching offers certain advantages over both alkaline hydrogen peroxide and hypochlorite, especially in that chlorite bleaching is extremely effective and economical. Chlorite bleaching shows a substantial improvement over either hydrogen peroxide or hypochlorite, particularly in retention of fiber strength, and provides the finisher with a strong fabric as the starting point for chemical finishing operations, for example, crease-proofing.

When bleaching with acidified chlorite solutions, however, it is necessary for the fibers to be in contact with the acidified solution containing an adequate amount of chlorite at a pH not above 4. When the aqueous chlorite solution is acidified to a pH of above 4 the bleaching action is not satisfactory. When the solution is acidified to a pH of about 4 or less, however, the solution is unstable on standing and an objectionable amount of chlorine dioxide gas is evolved. The chlorine dioxide gas is a powerful irritant to the eyes and respiratory systems of people. Furthermore, it represents a loss of bleaching power since the chlorite is being needlessly decomposed.

It is, therefore, an object of the present invention to provide a process for bleaching cellulosic textiles and textile fibers with acidified aqueous chlorite solutions.

It is a further object of the present invention to bleach cellulosic textiles and textile fibers in acidified aqueous chlorite solutions retaining the desirable characteristics of chlorite bleaching while obtaining improved brightness.

It is a still further object of the present invention to provide an aqueous chlorite bleaching bath which can be acidified to a pH of about 4 or less without objectionable chlorite decomposition and evolution of chlorine dioxide gas.

It is a still further object of the present invention to provide a process and aqueous acidic bleaching bath which accomplishes the foregoing objects inexpensively and expeditiously.

Further objects and advantages of the present invention will appear hereinafter.

The foregoing objects and advantages of the present invention may be accomplished in accordance with the present invention. The novel aqueous, acidic bleaching bath of the present invention has a pH of between 2 and 7 and comprises between about 0.1 and 3.0 percent by weight of a water soluble chlorite and between about 0.001 and 3.0 percent by weight of a water soluble hydrazine salt. Cellulosic textiles and textile fibers may be

2

effectively, inexpensively and expeditiously bleached by: wetting the textile to a pickup of 50 to 120 percent with acidified, aqueous chlorite solution having a pH of between 2 and 7 and comprising between about 0.1 and 3.0 percent by weight of a water soluble chlorite and between about 0.001 and 3.0 percent by weight of a water soluble hydrazine salt; holding the textile at a temperature between about 20 and 130° C. for between about 0.25 and 4 hours; and rinsing the textile in water.

It is surprising to find that the bleaching bath and process of the present invention produces improved bleaching over a bleach effected at the same pH without the hydrazine salt. This is especially surprising and unexpected in view of the normally vigorous reaction of concentrated solutions of hydrazine salts with concentrated solutions of chlorites and in view of the normally explosive reaction of dry hydrazine salts and dry chlorites. In addition it is surprising and unexpected to find that when the present invention is employed the bleaching solution may be kept at a pH of about 4 or below without the usual rapid decomposition of the chlorite and high incidence of objectionable chlorine dioxide evolution. Since the hydrazine salt inhibits the evolution of chlorine dioxide in the bleaching bath, the corrosion of stainless steel equipment, a serious problem in the art, is also markedly reduced.

Any water soluble chlorite may be employed. Alkali metal and alkaline earth metal chlorites are normally used, with the alkali metal chlorites being preferred. Sodium chlorite is especially preferred because it is commercially available in the form of "Textone," a product of Olin Mathieson Chemical Corporation containing about 80 percent sodium chlorite. Examples of suitable chlorites are lithium chlorite, potassium chlorite, sodium chlorite, calcium chlorite, barium chlorite and strontium chlorite.

Any water soluble hydrazine salt may be used in the process of the present invention, including partially substituted, water soluble hydrazine salts. Partially substituted hydrazine salts are those in which the hydrogen attached to the nitrogen of the hydrazine moiety is substituted by such groups as, for example, alkyl or aryl groups. Free hydrazine or partially substituted hydrazine may be added to the acidified solution, in which case the free hydrazine or the partially substituted hydrazine reacts with the acid to form the corresponding salt. The hydrazine salt may be either inorganic or organic. Typical hydrazine salts include, but are not limited to, the following: mineral acid salts such as, mono- or dihydrazine sulfate, mono- or dihydrazine phosphate, hydrazine mono- or dihydrochloride, hydrazine mono- or dihydribromide, hydrazine mono- or dihydroiodide, hydrazine borate and hydrazine carbazinate; aliphatic organic acid salts such as, alkane monobasic carboxylic acid salts, for example, hydrazine formate, hydrazine acetate and hydrazine propionate, alkene monobasic carboxylic acid salts, for example, hydrazine acrylate and hydrazine crotonate, alkyne monobasic carboxylic acid salts, for example, hydrazine propionate, saturated dibasic carboxylic acid salts, for example, mono- or dihydrazine oxalate, mono- or dihydrazine malonate, mono- or dihydrazine succinate and mono- or dihydrazine glutarate, unsaturated dibasic carboxylic acid salts, for example, mono- or dihydrazine maleate and mono- or dihydrazine fumarate, tribasic carboxylic acid salts, for example, mono-, di- or trihydrazine oxalate, mono-, di- or trihydrazine propane-1, 2,3-tricarboxylate and mono-, di- or trihydrazine citrate, alkane sulfonic acid salts, for example, hydrazine methyl sulfonate, hydrazine ethyl sulfonate and hydrazine propyl sulfonate, halogen or hydroxy substituted salts, for example, hydrazine mono-, di- or trichloroacetate, hydrazine glycolate, hydrazine lactate, hydrazine 2-hydroxypropionate, hydrazine mono- or dimalate and hydrazine mono- or ditartrate, and amino acid salts, for example, hydrazine aminoacetate, hydrazine 1-aminopropionate and hydrazine

1-aminovalerate; aromatic acid salts such as, hydrazine benzene sulfonate, hydrazine toluene sulfonate, hydrazine *p*-halobenzene sulfonate, mono- or dihydrazine benzene disulfonate, mono-, di- or trihydrazine benzene trisulfonate, hydrazine phenylsulfonate, hydrazine benzoate, hydrazine *ortho*-, *meta*- or *para*-chlorobenzoate, hydrazine *ortho*-, *meta*- or *para*-nitrobenzoate, hydrazine salicylate, hydrazine phenylacetate, mono- or dihydrazine phthalate, mono- or dihydrazine isophthalate, mono- or dihydrazine terephthalate, hydrazine cinnamate, hydrazine *o*-hydroxy-cinnamate, hydrazine naphthoate, hydrazine naphthalene sulfonate and hydrazine naphthenate; cycloaliphatic salts such as, hydrazine hexahydrobenzoate; and partially substituted hydrazine salts such as, mono-, di- or trihydroxy-alkyl-substituted hydrazine salts, mono- or trialkyl-substituted hydrazine salts, monoaryl-substituted hydrazine salts and mixed alkyl-aryl-substituted hydrazine salts. It is to be understood that mixtures of hydrazine salts may be advantageously employed in the process of the present invention. It is also to be understood that hydrazine salts containing mixed substituents may be advantageously employed in the process of the present invention.

The concentration of the chlorite in the aqueous solution may be varied from between about 0.1 and 3.0 percent by weight, with the concentration of the chlorite applied to the textile varying from between about 0.1 and 3.0 percent by weight based on the weight of the textile. Different types of textiles require different amounts of chlorite to effect a maximum whiteness. Thus a heavy linen may require twice as much as a light cotton. Those skilled in the art of bleaching are familiar with the requirements of various cellulosic textiles and textile fibers.

The concentration of the hydrazine salt in the aqueous solution may be varied from between about 0.001 and 3.0 percent by weight, and preferably between about 0.01 and 0.20 percent by weight. The amount of hydrazine applied to the textile is appropriately from between about 1 and 100 percent by weight of the chlorite, and preferably between about 5 and 25 percent by weight of the chlorite.

It is preferred to prepare a single solution containing the requisite amount of chlorite and hydrazine salt in the proper pH range, immerse the textile in the solution and remove the excess liquid. The textile may also be wetted by spraying the solution on the textile. Alternatively, two solutions may be prepared, with one solution being the aqueous chlorite solution and the other aqueous hydrazine salt solution. The textile may then be immersed successively in each solution and excess liquid removed after each immersion.

In the preferred process of the present invention the textile is immersed in an aqueous solution containing the requisite quantity of chlorite and hydrazine salt and acidified to a pH of between 2 and 7. The acid used for the acidification is not critical, for example, typical acids include formic, acetic, hydrochloric, sulfuric, phosphoric, or nitric. The textile is then removed from the solution and excess liquid removed so that the textile has a pickup of from 50 to 120 percent based on the weight of the textile. The excess liquid may be removed by, for example, passing through pre-set squeeze rolls.

After the textile has been wetted with the aqueous solution containing chlorite and hydrazine it is stored until bleaching is complete. This process is greatly accelerated by heat; a humid atmosphere at about 50 to 100° C. for 0.5 to 3 hours is excellent, although a temperature range of from 20 to 130° C. for from 0.25 to 4 hours may be employed. The humidity can be supplied by applying the heat in the form of steam in a steam box. The humidity may also be supplied by evaporation of a minor amount of the water on the textile if the textile is in a container of small volume which is quickly saturated with water vapor. The solution on the textile should not lose a material proportion of the water, however, since bleaching is preferably effected by dilute chlorite solutions.

After completion of the holding period the textile is rinsed in water and dried according to conventional procedures.

The bleaching solution may optionally contain various conventional additives which are stable to the components of the bleaching solution. The use of these additives will be apparent to one skilled in the art. Typical additives include the conventional buffers, such as sodium phosphate and sodium acetate, wetting agents, such as members of the "Igepon" series (salts of acylalkyl taurides), corrosion inhibitors, such as water soluble nitrate salts, and chelating agents such as, those amines having a plurality of hydrogen groups of the amino group replaced by fatty carboxylic acid groups.

The following examples will further illustrate the present invention and improvements obtained thereby.

#### EXAMPLES 1-16

In the following examples the textile was immersed in an acidified dilute solution containing 100 cc. of a two percent solution of sodium chlorite and the indicated amount of a two percent solution of the hydrazine salt. The textile was squeezed through pre-set squeeze rolls to a pickup of about 85 percent based on the weight of the textile. The textile was then heated in a steam box at 110 to 120° C. for about one hour, rinsed thoroughly in water and dried. None of the textiles treated showed any signs of textile damage. The reflectance was measured with a Photovolt Brightness Meter equipped with a tristimulus blue filter. With the brightness scale used a difference of two units is noticeable to the unaided eye, while a difference of ten units represents a striking difference in whiteness. In the brightness range above 80 it becomes increasingly difficult to obtain each additional point of brightness without damage to the textile; therefore, the improvements shown in the following examples are of particular commercial importance.

The following examples utilized a greige cotton textile having an initial whiteness of 52. When this textile was treated in the above manner in a solution acidified to a pH of 3.5 but which did not contain a hydrazine salt the brightness was 85.

In the following examples the following abbreviations are used:

MHS=monohydrazine sulfate  
DHS=dihydrazine sulfate  
DHP=dihydrazine phosphate  
MHN=monohydrazine nitrate  
HA=hydrazine acetate

Table I

| Example | c.c. of a 2% Solution of Hydrazine Salt | c.c. of a 2% Solution of Sodium Chlorite | cc. of Water | pH of Solution | Brightness |
|---------|-----------------------------------------|------------------------------------------|--------------|----------------|------------|
| 1       |                                         | 100                                      | -----        | 3.5            | 85.0       |
| 2       | 5 cc. MHS                               | 100                                      | -----        | 6.3            | 88.4       |
| 3       | 6 cc. MHS                               | 100                                      | -----        | 4.9            | 88.5       |
| 4       | 7 cc. MHS                               | 100                                      | -----        | 4.1            | 88.9       |
| 5       | 6.34 cc. DHS                            | 100                                      | 85           | 6.5            | 87.0       |
| 6       | 6.34 cc. DHS                            | 100                                      | 85           | 5.5            | 87.6       |
| 7       | 6.34 cc. DHS                            | 100                                      | 85           | 4.5            | 88.1       |
| 8       | 6.34 cc. DHS                            | 100                                      | 85           | 3.5            | 88.5       |
| 9       | 6.34 cc. DHP                            | 100                                      | 80           | 5.5            | 88.5       |
| 10      | 6.34 cc. DHP                            | 100                                      | 80           | 4.5            | 88.9       |
| 11      | 8.24 cc. MHN                            | 100                                      | 80           | 6.5            | 88.0       |
| 12      | 8.24 cc. MHN                            | 100                                      | 80           | 5.5            | 88.6       |
| 13      | 8.24 cc. MHN                            | 100                                      | 80           | 4.5            | 88.2       |
| 14      | 8.24 cc. MHN                            | 100                                      | 80           | 3.5            | 89.0       |
| 15      | 7.2 cc. HA                              | 100                                      | 80           | 5.5            | 87.8       |
| 16      | 7.2 cc. HA                              | 100                                      | 80           | 4.5            | 89.0       |

#### EXAMPLES 17-18

In the following examples the procedure of Examples 1-16 was repeated, except that the textile was heated in a steam box at 94 to 97° C. for 30 minutes. There were no signs of textile damage.

**5**  
*Table II*

| Example | cc. of a 2%<br>Solution of<br>Monohy-<br>drazine<br>Nitrate | cc. of a 2%<br>Solution of<br>Sodium<br>Chlorite | cc. of<br>Water | pH of<br>Solution | Brightness |
|---------|-------------------------------------------------------------|--------------------------------------------------|-----------------|-------------------|------------|
| 17..... | 8.24                                                        | 100                                              | 80              | 4.5               | 84.5       |
| 18..... |                                                             | 100                                              | 80              | 4.5               | 74.5       |

**EXAMPLES 19-25**

In the following examples the procedure of Examples 1-16 was repeated, except that the bleaching solution contained 2.5 grams per liter of sodium chlorite and dihydrazine phosphate as indicated and the textile was heated in a steam box for one hour at 210° F. There were no signs of textile damage.

*Table III*

| Example | Grams per<br>Liter of<br>Dihydra-<br>zine Phos-<br>phate | Grams per<br>Liter of<br>Sodium<br>Chlorite | pH of Solu-<br>tion | Brightness |
|---------|----------------------------------------------------------|---------------------------------------------|---------------------|------------|
| 19..... | 0.16                                                     | 2.5                                         | 7.0                 | 75.0       |
| 20..... |                                                          | 2.5                                         | 7.0                 | 72.5       |
| 21..... | 0.16                                                     | 2.5                                         | 6.0                 | 84.5       |
| 22..... |                                                          | 2.5                                         | 6.0                 | 79.5       |
| 23..... | 0.16                                                     | 2.5                                         | 5.0                 | 87.1       |
| 24..... |                                                          | 2.5                                         | 5.0                 | 81.5       |
| 25..... |                                                          | 2.5                                         | 3.0                 | 87.5       |

**EXAMPLES 26-31**

Aqueous solutions were prepared in a manner after Examples 1-16 and the stability of the solution measured. The stability was measured by observing the length of time it took for the solution to become perceptibly yellow and actively evolve a strong odor of chlorine dioxide.

*Table IV*

| Example | cc. of a 2%<br>Solution of<br>Hydrazine Salt | cc. of a 2%<br>Solution of<br>Sodium<br>Chlorite | cc. of<br>Water | pH of<br>Solution | Stability<br>Hours |
|---------|----------------------------------------------|--------------------------------------------------|-----------------|-------------------|--------------------|
| 26..... |                                              | 100                                              | 85              | 3.5               | 0.25               |
| 27..... | 6.34 cc. DHS                                 | 100                                              | 85              | 6.5               | 20                 |
| 28..... | 6.34 cc. DHS                                 | 100                                              | 85              | 3.5               | 1>7                |
| 29..... | 6.34 cc. DHP                                 | 100                                              | 80              | 4.5               | 1>8                |
| 30..... | 6.34 cc. DHP                                 | 100                                              | 80              | 3.5               | 1>4                |
| 31..... | 8.24 cc. MHN                                 | 100                                              | 80              | 6.5               | 1>24               |

<sup>1</sup> Test discontinued after this time.

This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

What is claimed is:

1. A process for bleaching cellulosic textiles and textile fibers which comprises: wetting the textile to a pickup of 50 to 120 percent with acidified, aqueous chlorite solution having a pH of between 2 and 7 and comprising be-

**6**

tween 0.1 and 3.0 percent by weight of a water soluble chlorite and between 0.001 and 3.0 percent by weight of a water soluble hydrazine salt; holding the textile at a temperature of between 20 and 130° C. for between 0.25 and 4 hours; and rinsing the textile in water.

2. A process for bleaching cellulosic textiles and textile fibers which comprises: wetting the textile with an acidified, aqueous solution having a pH of between 2 and 7 comprising water soluble chlorite to apply to the textile

10 between 0.1 and 3.0 percent of said chlorite by weight of the textile; further wetting said textile with an aqueous solution comprising water soluble hydrazine salt to apply to the textile between 1 and 100 percent of said hydrazine salt by weight of the chlorite; holding the textile at a 15 temperature of between 20 and 130° C. for between 0.25 and 4 hours; and rinsing the textile in water.

3. A process for bleaching cellulosic textiles and textile fibers which comprises: immersing the textile in an acidified, aqueous solution having a pH of between 2 and 7

20 and comprising between from 0.1 to 3.0 percent by weight of a water soluble chlorite and between 0.001 and 3.0 percent by weight of a water soluble hydrazine salt; squeezing the textile to a pickup of 50 and 120 percent; holding the textile at a temperature of between 20 and 130° C. for between 0.25 and 4 hours; and rinsing the textile in water.

4. A process according to claim 3 wherein the chlorite is sodium chlorite.

5. A process according to claim 4 wherein the hydrazine salt is monohydrazine sulfate.

6. A process according to claim 4 wherein the hydrazine salt is dihydrazine sulfate.

7. A process according to claim 4 wherein the hydrazine salt is dihydrazine phosphate.

35 8. A process according to claim 4 wherein the hydrazine salt is monohydrazine nitrate.

9. A process according to claim 4 wherein the hydrazine salt is hydrazine acetate.

10. An aqueous, acidic bleaching bath having a pH of 40 between 2 and 7 comprising between 0.1 and 0.3 percent by weight of a water soluble chlorite and between 0.001 and 3.0 percent by weight of a water soluble hydrazine salt.

11. The aqueous, acidic bleaching bath of claim 10 wherein said chlorite is sodium chlorite.

12. The aqueous bleaching bath of claim 11 wherein said hydrazine salt is monohydrazine sulfate.

13. The aqueous bleaching bath of claim 11 wherein said hydrazine salt is dihydrazine sulfate.

50 14. The aqueous bleaching bath of claim 11 wherein said hydrazine salt is dihydrazine phosphate.

15. The aqueous bleaching bath of claim 11 wherein said hydrazine salt is monohydrazine nitrate.

16. The aqueous bleaching bath of claim 11 wherein said hydrazine salt is hydrazine acetate.

**References Cited in the file of this patent**

**UNITED STATES PATENTS**

60 2,947,700 Waibel ----- Aug. 2, 1960

**OTHER REFERENCES**

Mosse: Teintex, November 15, 1954, pp. 811-812.